

# UNITED STATES PATENT OFFICE.

WILLIAM CAMPBELL, OF NEW YORK, N. Y., JOHN H. HALL, OF HIGH BRIDGE, NEW JERSEY, AND HENRY M. HOWE, OF BEDFORD STATION, NEW YORK, ASSIGNEES TO TAYLOR-WHARTON IRON AND STEEL COMPANY, A CORPORATION OF NEW JERSEY.

## MANUFACTURE OF MANGANESE STEEL.

1,113,539.

Specification of Letters Patent. Patented Oct. 13, 1914.

No Drawing.

Application filed August 10, 1908. Serial No. 447,742.

To all whom it may concern:

Be it known that we, WILLIAM CAMPBELL, a subject of His Majesty the King of England, and a resident of the city, county, and State of New York, JOHN H. HALL, a citizen of the United States, and a resident of High Bridge, New Jersey, and HENRY M. HOWE, a citizen of the United States, and a resident of Bedford Station, Westchester county, New York, have invented certain new and useful Improvements in the Manufacture of Manganese Steel, of which the following is a full, true, and concise specification.

This invention is an improvement in manganese steel alloys, and provides a new class of such alloys possessing the characteristic hardness and toughness of existing forms of manganese steel but containing a lower percentage of manganese, which feature adapts the new product for production at a less cost and affords practical advantages in certain other respects.

Manganese steel as now made and used contains usually from 11 to 14 per cent. manganese, and from 1 to 1.5 per cent. of carbon, and is characterized not only by its remarkable combination of hardness and toughness or ductility, but also by the peculiarity that it is made malleable by quenching it, when heated, in a cold liquid. We are aware that it has been hitherto proposed to employ smaller percentages of manganese, but a manganese steel, low in manganese, has not yet been produced of commercial or satisfactory character, and we believe it is generally conceded that reduction of the manganese below the above percentage, or say 10 per cent., produces or tends to produce a brittleness in the product akin to the brittleness of glass, which unfit it for practical or commercial use.

Our invention is based on the discovery we have made, that a certain critical relation exists between the percentage of manganese and the percentage of carbon employed with it in the alloy, and that by proportioning the carbon ingredient in accordance with this relation, a product steel may be obtained containing comparatively small percentages of manganese, say from 9 per cent. to 6 per cent. or as low as 5 per cent. and possessing to a very valuable degree the

characteristic combination of ductility with hardness and the other well known and important properties of the richer alloys. As the percentage of manganese is diminished below about 6 per cent., we observe that the peculiar properties that are characteristic of manganese steel begin to disappear, as if approaching the region where manganese steel merges into ordinary carbon steel, which, as is known, contains manganese in minute amounts, but of which the properties are quite opposite. There is therefore, as we believe, a practical limit, around 5 per cent., for the diminution of the manganese according to our invention.

The relation we have found to exist between the percentages of manganese and carbon may be expressed by a statement, as follows, of the limits within which the carbon may be usefully present in steel containing from 9 to 5 per cent. or thereabout of manganese, viz. an amount equal to  $.985 - .04$  of the percentage of manganese as one limit, and an amount equal to  $1.25 + \frac{1}{4}$  of the percentage of manganese as the other limit, the particular amount of carbon between these limits for any given percentage of manganese being determined according to the degree of ductility desired for the product. Thus, for example, if an 8 per cent. manganese steel be required, the carbon is introduced in such amounts that the finished product will contain between  $(.985 - .04) \times 8 = .665\%$  and  $(1.25 + \frac{1}{4} \times 8) = 1.516\%$  in percentage of the whole, and if the product be required to be specially ductile, the amount of carbon present should be nearer the lower of the two limits,—the carbon referred to being carbon other than graphite.

As the carbon content approaches the extremes of its range, as above determined, however, we find an increasing tendency toward brittleness and lack of uniformity in the product, due to an apparent instability of its molecular arrangement and the disproportionate effects of slight variations in its treatment, and for this reason we prefer and recommend a somewhat narrower range wherein the carbon may be introduced in such variable amounts as still to afford some control of the character of the resultant product, but with practically no danger of

retrogression of the metal into unserviceable forms.

By way of explanation, it may be said that the slower the cooling of a casting containing extreme percentages of carbon, the greater is the tendency toward retrogression into undesirable brittleness and such brittleness is most apt to occur in thick pieces, the interior of which necessarily cools rather slowly. Other causes also, which need not be here explained, are believed to exaggerate this tendency. In its preferred form, therefore, our product having in its composition an amount of manganese less than 9 per cent. and somewhat more than 5 per cent. contains carbon, other than graphite, between or not materially exceeding the following narrower limits, viz. 1.075-.04 of the percentage of manganese as one limit, and 1.075+ $\frac{1}{3}$  of the percentage of manganese as the other limit, the percentages being taken with reference to the whole. For example, for an 8 per cent. manganese steel the preferable limits for the carbon are (1.075-.04×8)=.755% and (1.075+ $\frac{1}{3}$ ×8)=1.342%, the particular amount of carbon present being controlled within these limits as before and according to the degree of ductility required in the product.

The ingredients of the product are preferably measured and brought together in a molten state, as is now usual with manganese-steel alloys, and in the proportions above stated, and after casting, the product is to be properly water-toughened, which may be done by heating and suddenly cooling it, as by quenching in cold water from a temperature of say 1070° centigrade or between 1010° and 1110° C. or thereabout, whereby the product will appear, under a magnification of say 100 diameters, as a homogeneous substance, or composed of a single constituent as distinguished from a composite or conglomerate of several visibly distinct substances. In its physical properties, the new alloy is characterized by its ductility and hardness as above stated, and by the fact that it is a poor conductor of heat, and is practically non-magnetic.

It will, of course, be understood that certain other elements may be present in the product in small quantities, as is generally the case with steel alloys, without departing from this invention.

Having described our invention, what we

claim and desire to secure by Letters Patent of the United States, is:

1. A manganese steel alloy containing from nine to five per cent. of manganese and containing carbon within the following limits, viz., substantially 1.075 per cent. minus .04 of the percentage of manganese as one limit and 1.25 per cent. plus  $\frac{1}{3}$  of the percentage of manganese as the other limit, and having the qualities of ductility and hardness substantially as described.

2. A manganese steel alloy containing from 9 to 6 per cent. manganese and containing carbon in an amount not exceeding the following limits, viz: 1.075 per cent. minus .04 of the percentage of manganese as one limit, and 1.075 per cent. plus  $\frac{1}{3}$  of said percentage of manganese as the other limit.

3. A manganese steel alloy containing from 9 to 6 per cent. manganese and having combined therewith an amount of carbon not substantially exceeding the following limits, viz: 1.075 per cent. minus .04 of the percentage of manganese as one limit and 1.075 per cent. plus  $\frac{1}{3}$  of said percentage of manganese as the other limit, said alloy being practically non-magnetic, and characterized by ductility combined with hardness.

4. A manganese steel alloy containing less than 9 per cent. manganese and containing carbon within the following limits, viz: 1.075 per cent. minus .04 of the percentage of manganese as one limit, and 1.075 per cent. plus  $\frac{1}{3}$  of the percentage of manganese as the other limit, said alloy being practically non-magnetic and presenting the appearance of a homogeneous substance when magnified to 100 diameters and having the characteristic of hardness combined with ductility.

In testimony whereof, we have signed our names to the specification in the presence of two subscribing witnesses.

WILLIAM CAMPBELL.  
JOHN H. HALL.  
HENRY M. HOWE.

Witnesses as to W. Campbell:

A. P. FRAPWELL,  
R. G. WILLIAMS.

Witnesses as to J. H. Hall:

H. G. KIMBALL,  
G. A. TAYLOR.

Witnesses as to H. M. Howe:

EDWARD C. GROESBECK,  
HELEN M. TOWEY.